

Patented July 21, 1953

2,646,426

# UNITED STATES PATENT OFFICE

2,646,426

## PREPARATION OF PHOTOGRAPHIC EMULSIONS

Rudolph E. Damschroder, Rochester, N. Y., assignor to Eastman Kodak Company, Rochester, N. Y., a corporation of New Jersey

No Drawing. Application December 31, 1948,  
Serial No. 68,743

3 Claims. (Cl. 95—7)

1

This invention relates to methods of preparing photographic silver halide emulsions and more particularly to a process of forming photographic emulsions wherein by-products are removed for example by means of vacuum.

It is well known in the art of photographic emulsion making that it is desirable to remove soluble salts resulting from the emulsion making reactions especially in those cases where the emulsion is designed for coating on transparent supports. Equally well known are emulsions of the type where ammonia is used in making the emulsion and is present in the reaction mixture after formation of the silver halide. In such processes the ammonia and any soluble salt present is customarily removed by shredding the emulsion and washing with water by osmosis.

In such processes it is customary in the art, after precipitation of silver halide in the presence of a protective colloid, to chill the emulsion so that it can be cut up and shredded following which the pieces are washed for the desired time to remove salts or dissolved material such as ammonia. Frequently this process requires many hours to effect the removal of salt, and is performed in batches in crocks, tanks, shredding machines and other equipment for chilling, shredding and washing the emulsion.

It is, therefore, one object of my invention to provide a new method of making a photographic emulsion. Another object is to provide novel methods of making and purifying a photographic emulsion as by means of vacuum. A still further object is to provide an economical process of forming a photographic emulsion of optimum quality. Further objects of my invention will become apparent from consideration of the following description.

My invention resides in, and the objects are accomplished by, reaction of an aqueous ammoniacal solution of a silver compound with an ammonium or alkyl-ammonium halide so that the reaction products include silver halide, and other materials most of which are completely volatile. The reaction of the silver compound with the halide is carried out in the presence of a peptizing lyophilic colloid, e. g. gelatin.

It will be apparent that when I use vacuum for removal of a volatile material dissolved in a reaction mixture, a very economical process is made available. I have found that when vacuum is employed to remove ammonium compounds or other volatile compound from the emulsions of my invention, a decided saving in time, materials and manpower is effected. Also the photographic quality obtainable from the emulsion so treated is comparable to that obtainable by the washing technique of the prior art. The quality of the product can be higher especially since there is no possibility of emulsion contamination by impurities of wash water usually used.

2

The above advantages will become more apparent by consideration of the following detailed description of my invention.

The new type of emulsion reactions which are used involves reacting a silver compound such as silver oxide preferably but not necessarily dissolved in an excess of ammonia, with an ammonium or alkyl substituted ammonium halide of the following structure:



where X is a halogen atom and R, R<sub>1</sub> and R<sub>2</sub> each represent a hydrogen atom, or an alkyl group having from one to three carbon atoms, and in which the sum of the carbon atoms in R, R<sub>1</sub> and R<sub>2</sub> is not over three. Compounds having the above generic structure which I can use are the common ammonium halides, for example, ammonium chloride, bromide, or iodide and substituted ammonium halides, such as methyl ammonium bromide or chloride, dimethyl or trimethyl ammonium halides, and ethyl ammonium bromide or chloride. I can use one or more of such halides together and particularly in conjunction with an ammonium iodide. Generally, the total number of carbon atoms in the alkyl group or alkyl groups attached to the nitrogen atom in the above formula is less than four because the amines of more carbon atoms resulting from the emulsion reaction, are either too insoluble to be readily removed by washing or are not sufficiently volatile to be removed by vacuum or passing a current of air over the reaction mixture. Accordingly, I prefer to use ammonium or methyl ammonium halides in my invention.

The following examples are given as illustrative of my invention:

### Example 1

Silver oxide was made in the well-known manner by dissolving a quantity of silver nitrate in water and treating with excess sodium hydroxide solution until the silver oxide precipitated. The precipitate was separated, and washed by decantation. 0.125 mol of the resultant silver oxide was dissolved in a 10 per cent excess of aqueous ammonia and run into a solution containing 0.3 mol of ammonium bromide, 0.007 mol of ammonium iodide, 4 grams of gelatin and 130 cc. of water at 40° C. Precautions should be taken in dissolving the oxide in ammonia due to the explosive nature of the resultant silver complex. This may be accomplished by keeping the reaction product moist at all times. The reaction mixture now containing silver halide, ammonia, the excess ammonium bromide and water, was passed through an evacuated chamber as a thin film of liquid at a rate and under a pressure such that

only about 22 grams of ammonia remained associated with each kilogram of silver nitrate used in the reaction and converted to silver halide. The emulsion is now ready for addition of gelatin or other protein vehicle or other materials of similar property such as hydrolyzed cellulose esters or polyvinyl alcohol, and ripening or digesting operations or other steps customary in the art exclusive of washing may now be carried out.

*Example 2*

The silver oxide is made in the usual manner by precipitating it in a solution of aqueous silver nitrate by excess aqueous sodium hydroxide. The supernatant liquid is decanted and the precipitate is washed three times by distilled water. 0.125 mol of moist silver oxide is dissolved by 88 cc. of 28% ammonia in 100 cc. of water and the whole is diluted to 380 cc. This solution is run into a solution of 0.264 mol of ammonium bromide, 0.0053 mol of potassium or ammonium iodide and 6.1 gm. of gelatin in 380 cc. of water. The resulting mixture which contains silver halide, ammonia and excess ammonium bromide is passed through a vacuum still in which the temperature and pressure are regulated such that the emulsion emerging from the still has a pH of 8.5 or less. Gelatin is added to the emulsion, the pH is adjusted by dilute sulfuric acid and dilute silver nitrate is added and then the emulsion is finished and coated by methods customary in the art exclusive of washing.

In some cases in the examples herein, it is desirable to dissolve the silver oxide in aqueous ammonia solution in the presence of a colloidal material such as gelatin, e. g., about 0.1% gelatin in the solution, and in those instances when prohibitive fog results from so doing, fog may be diminished by addition of from about 0.5 to 2.5 mg. of potassium permanganate per gram of gelatin. To the emulsion thus treated may then be added the usual emulsion addenda, gelatin, sensitizers, etc., and finished in the usual manner exclusive of washing.

*Example 3*

The procedure of Example 2 is followed with the exception that the ammonia used for the conversion of silver oxide is replaced by 200 cc. of approximately 25% aqueous methylamine which yields an "ammoniacal" solution of the silver compound. The mixture obtained by adding this solution to the salts contains ammonia, excess ammonium bromide and methylamine. The ammonia and methylamine are removed in the vacuum still at a temperature and pressure such that the collected emulsion has a pH of 8.5 to 9 or lower. The emulsion is then treated by the customary procedures exclusive of washing.

*Example 4*

The method of using an alkyl substituted ammonium halide instead of ammonium halide in my process is as follows:

The procedure of Example 2 is followed with the exception that the ammonium bromide is replaced by an equivalent quantity of trimethyl ammonium bromide. The trimethyl ammonium bromide is prepared by treating trimethylamine with aqueous hydrobromic acid. The mixture resulting from adding this solution to the salts contains silver halide, ammonia, excess trimethyl ammonium bromide and trimethylamine. The ammonia and the trimethylamine are removed in the vacuum still such that the pH of the re-

sulting emulsion is 8.5 to 8.9 or lower. The emulsion is further treated by the customary methods exclusive of washing.

*Example 5*

A silver salt such as silver carbonate may be employed in making my emulsions as follows:

Silver carbonate is prepared by treating an aqueous solution containing 0.25 mol of silver nitrate with excess sodium carbonate. The supernatant liquid is decanted and the precipitate is washed three times by distilled water. This is converted by adding 45 cc. of 28% ammonia and the resulting solution is diluted to 380 cc. This solution is run into a solution of halides containing the same quantities of materials as in Example 2. The resulting mixture contains silver halide, ammonia, excess ammonium bromide and ammonium carbonate, and is passed through the vacuum still by which the ammonia and the ammonium carbonate are removed until the emerging emulsion has a pH of 8.5 or less. The emulsion is then treated by the customary methods exclusive of washing.

The emulsions made by the above procedures have a speed, gamma and graininess such that they are usable for fine grain negative emulsions.

*Example 6*

The process outlined in Example 2 is followed with the exception that the gelatin is replaced with equivalent quantities of a water-soluble oxidized protein or protein derivative such as disclosed in the co-pending Lowe et al. U. S. patent application Serial No. 768,480, filed August 13, 1947, e. g. the acrylonitrile-acetyl derivative of oxidized casein.

In the above examples, the volatile by-products resulting are removed by evacuation or by passing a stream of air over the mixture. Also, it will be noted that in the above examples the silver compounds were reacted with a slight excess of halide in order that the resultant reaction mixture will contain silver halide, volatile nitrogen compound and the excess halide; however, for the purposes of my invention this excess of halide is not considered to be appreciable and the reaction mixture may be said to contain, substantially no non-volatile by-product. If desired, I can, in the above examples employ equivalent amounts of silver and halide compounds and produce useful emulsions in the manner of my invention.

The peptizing lyophilic colloids which I use during the step of precipitating the silver halide, are materials such as gelatin, polyacrylamide or imide resins such as disclosed in Lowe et al. U. S. application, Serial No. 685,375, filed July 22, 1946, now Patent No. 2,541,474; casein, modified proteins such as disclosed in Lowe et al. U. S. application, Serial No. 768,480, filed August 13, 1947, and similar materials.

In order to remove the ammonia from the emulsion systems I describe, I have found it advisable to supply heat to the liquid being evacuated to compensate for the drop in temperature arising from the heat supplied for vaporization and the tendency for the rate of removal of ammonia to fall with drop in temperature thereby. The rate and extent of the removal of moist ammonia is, of course, controlled on the one hand by the peculiarities of the vacuum equipment and the flow of the liquid through it which naturally depends in some degree upon the capacity of the vacuum pumping means. A useful range of

operation includes a range of pressure in the vacuum system of from 20 to 30 mm. of mercury or lower and when heat is supplied to the liquid film by means of a water jacket a range of temperature from 60 to 80° C. in the jacket is satisfactory. However, in a typical all-glass installation using water jackets and aspirator pumps, appreciable amounts of ammonia are removed with the water at 40° C. and a vacuum pressure of 90 mm. As is apparent, the most suitable or desirable conditions of rate of flow, temperature and pressure for a given apparatus are readily determinable but depend on definite characteristics of that equipment. After I determine the characteristics of the vacuum system, that is, its rate of removal of ammonia or dissolved material, I am next governed by matters of economy and photographic quality. That is, in certain instances where it is desired to remove substantially all of the ammonia from the reaction mixture, I can do so by selection of the optimum conditions of temperature, pressure and rate of flow through the evacuation chamber. In other cases where I have use for an emulsion from which all of the ammonia has not been removed, I naturally increase the rate of flow or lower the temperature or increase the pressure or I can vary one or more of these conditions at the same time as will be apparent to those skilled in the art.

Since the grain characteristics and photographic properties of an ammoniacal emulsion are controlled by the concentration, temperature and time of the ammonia solutions in contact with the silver salt, it is desirable to operate my invention in such a way that the grains of silver salt are ripened and the ammonia is reduced in concentration to less than 22 grams per kilogram of silver nitrate converted to silver halide in a total time of less than 2 hours. This I may accomplish either by short ripening and slow removal or by more prolonged ripening and fast removal or short ripening and fast removal.

One advantage of my process is now apparent. Having determined the operating characteristics of the emulsion making system I may remove practically any quantity of ammonia or volatile material from the silver halide reaction mixture. If I desire an emulsion having all of the characteristics derivable from a similar well-washed emulsion, I remove that amount of ammonia which corresponds to washing. Similarly, if desired, I remove less ammonia with the result, among other things, of obtaining an appreciable increase in the output of the evacuation system. Since sensitometric characteristics and photographic quality are of prime importance, I remove an amount of ammonia commensurate with utmost economy and proven dictates of photographic quality.

Finished emulsions having desirable photographic qualities can be made by removing ammonia until a range of from about 0 to 22 grams of ammonia per kilogram of silver nitrate (5.9 mols of silver nitrate or 2.95 mols calculated as silver oxide or silver carbonate) used in making the emulsion and converted to silver halide remains associated with the silver halide. That is, the volatile nitrogen compounds present in the reaction mixture are removed until the molecular equivalent of the nitrogen compound remaining in the emulsion is equal to less than about 22 grams of ammonia per kilogram of silver nitrate used.

It will be apparent that when an alkyl substituted ammonium halide is used, for example,

according to Example 4, the efficiency of my process may be lowered principally because of the higher boiling point of the aliphatic amine formed in the reaction and which is to be removed from the reaction mixture. In such cases I may desire to wash the material from the emulsion with or without previous evacuation treatment as I can do when ammonium halides are used.

In certain cases it may be desirable to carry out the evacuation of the emulsion before, or after, ripening or digesting or other steps known to emulsion making. However, I prefer to remove a material such as ammonia prior to ripening of the emulsion. My process is especially adaptable to removing the ammonia just after or as soon after formation of silver halide as is possible and therefore may be readily adapted to a continuous manufacturing process. I merely conduct the silver halide reaction mixture in a continuous manner from the reaction chamber to the evacuation chamber and if the evacuation system is operated at a fairly low capacity, I use a temporary holding tank therebetween. An advantage of the quick removal of ammonia or amine lies in the fact that the emulsion has no appreciable opportunity to ripen in the presence of an undesirable quantity of ammonia or amine, and it is removed much more quickly than by washing. Therefore, silver halide grain size can be controlled more readily than previously by operating according to my invention.

It is to be noted that when the composition resulting from my process is ripened or digested or treated as usual, the finished emulsion has as good characteristics as it would have had, had washing been employed. There is thus made available a process whereby I can remove all or a part of the ammonia associated with the silver halide, then can if desired add definite quantities of ammonia during finishing operations, but I am not limited, contrary to washing methods, to grain characteristics obtained while silver halide is in contact with ammonia during a chilling period prior to and including washing.

It is to be understood that the disclosure herein is by way of example and I consider as included in my invention all modifications and equivalents falling within the scope of the appended claims.

What I claim is:

1. A method of making a photographic silver halide emulsion which comprises reacting in an excess of aqueous ammoniacal solution substantially free of nitrate ion in the presence of a peptizing hydrophilic colloid for silver halide, substantially equivalent molar quantities of a compound selected from the group consisting of silver oxide and silver carbonate with at least one of the amine halides having the formula



wherein X represents a halogen atom, R, R<sub>1</sub> and R<sub>2</sub> each represents a member selected from the group consisting of a hydrogen atom and an alkyl group having from 1 to 3 carbon atoms, the sum total of the carbon atoms in R, R<sub>1</sub> and R<sub>2</sub> being from 0 to 3, to yield a silver halide emulsion containing silver halide, a volatile nitrogen compound and substantially no other non-volatile product, removing said volatile nitrogen compound from said emulsion only by passing the emulsion as a thin film of liquid through a chamber maintained at a pressure of about 20-90

mm. of mercury and a temperature of from about 40-80° C. until the molecular equivalent amount of the nitrogen compound remaining in the emulsion is equal to less than about 22 grams of ammonia per 2.95 mols of said silver compound selected from the group consisting of silver oxide and silver carbonate used in making the emulsion and converted to silver halide, and digesting the emulsion, the removal of nitrogen compound and digestion being effected within less than two hours.

2. A method of making a photographic silver halide emulsion which comprises reacting in excess aqueous ammonia solution substantially free of nitrate ion in the presence of gelatin, substantially equivalent molar quantities of silver oxide and an ammonium halide to yield a silver halide emulsion containing silver halide, ammonia and substantially no other non-volatile product, removing the ammonia from the emulsion only by passing the emulsion as a thin film of liquid through a chamber maintained at a pressure of from about 20 to 90 mm. of mercury and a temperature of from about 40-80° C. until the amount of ammonia remaining in the emulsion is equal to less than about 22 grams of ammonia per 2.95 mols of silver oxide used in making the emulsion and converted to silver halide, and digesting the emulsion, the removal of ammonia and digestion being effected within less than two hours.

3. A method of making a photographic silver halide emulsion which comprises reacting in excess aqueous ammonia solution substantially free of nitrate ion in the presence of gelatin, substantially equivalent molar quantities of silver carbonate and an ammonium halide to yield a silver

10

15

20

25

30

35

halide emulsion containing silver halide, ammonia and substantially no other non-volatile product, removing the ammonia from the emulsion only by passing the emulsion as a thin film of liquid through a chamber maintained at a pressure of from about 20 to 90 mm. of mercury and a temperature of from about 40-80° C. until the amount of ammonia remaining in the emulsion is equal to less than about 22 grams of ammonia per 2.95 mols of silver carbonate used in making the emulsion and converted to silver halide, and digesting the emulsion, the removal of ammonia and digestion being effected within less than two hours.

18

RUDOLPH E. DAMSCHRODER.

## References Cited in the file of this patent

## UNITED STATES PATENTS

| Number    | Name           | Date           |
|-----------|----------------|----------------|
| 1,861,918 | Hickman        | July 7, 1932   |
| 2,158,219 | Claus          | May 16, 1939   |
| 2,256,356 | Russell et al. | Sept. 16, 1941 |
| 2,403,327 | Baker          | July 2, 1946   |

## FOREIGN PATENTS

| Number  | Country       | Date          |
|---------|---------------|---------------|
| 3,782   | Great Britain | 1873          |
| 477,315 | Great Britain | Mar. 23, 1936 |

## OTHER REFERENCES

- Wall, "Photographic Emulsions," published by American Photographic Publishing Co., 1929, pp. 221, 222, 223, 225 and 226 cited, pp. 158-161.  
 The Amateur Photographer, vol. 18, pp. 223, 224, 242, and 243.